



US008728693B2

(12) **United States Patent**  
**Hamano et al.**

(10) **Patent No.:** **US 8,728,693 B2**  
(b5) **Date of Patent:** **\*May 20, 2014**

(54) **TONER FOR DEVELOPING ELECTROSTATIC IMAGE, METHOD OF PRODUCING TONER, CARTRIDGE, IMAGE FORMING METHOD, AND IMAGE FORMING APPARATUS**

(75) Inventors: **Hirokazu Hamano**, Kanagawa (JP); **Tetsuya Taguchi**, Kanagawa (JP); **Asafumi Fujita**, Kanagawa (JP); **Hiroshi Kamada**, Kanagawa (JP); **Masahiro Takagi**, Kanagawa (JP)

(73) Assignee: **Fuji Xerox Co., Ltd.**, Tokyo (JP)

(\*) Notice: Subject to any disclaimer, the term of this patent is extended or adjusted under 35 U.S.C. 154(b) by 38 days.

This patent is subject to a terminal disclaimer.

(21) Appl. No.: **13/234,879**

(22) Filed: **Sep. 16, 2011**

(65) **Prior Publication Data**

US 2012/0251936 A1 Oct. 4, 2012

(30) **Foreign Application Priority Data**

Mar. 28, 2011 (JP) ..... 2011-070899

(51) **Int. Cl.**  
**G03G 9/00** (2006.01)

(52) **U.S. Cl.**  
USPC ..... 430/108.6; 430/108.1; 430/108.7

(58) **Field of Classification Search**  
USPC ..... 430/108.1, 108.6, 108.7  
See application file for complete search history.

(56)

**References Cited**

**U.S. PATENT DOCUMENTS**

|                   |         |                       |           |
|-------------------|---------|-----------------------|-----------|
| 7,160,662 B2 *    | 1/2007  | Yoshino et al. ....   | 430/108.3 |
| 7,354,688 B2 *    | 4/2008  | Silence et al. ....   | 430/108.3 |
| 7,485,400 B2 *    | 2/2009  | Veregin et al. ....   | 430/107.1 |
| 7,537,876 B2      | 5/2009  | Anno et al.           |           |
| 2003/0118929 A1   | 6/2003  | Shirai et al.         |           |
| 2007/0009823 A1 * | 1/2007  | Skorokhod et al. .... | 430/108.3 |
| 2009/0035683 A1 * | 2/2009  | Imafuku et al. ....   | 430/108.7 |
| 2012/0251937 A1 * | 10/2012 | Fujita et al. ....    | 430/105   |

**FOREIGN PATENT DOCUMENTS**

|                  |         |
|------------------|---------|
| JP A-49-091231   | 8/1974  |
| JP A-56-040868   | 4/1981  |
| JP A-2003-005436 | 1/2003  |
| JP A-2003-107781 | 4/2003  |
| JP A-2004-053710 | 2/2004  |
| JP A-2004-086005 | 3/2004  |
| JP A-2004-109200 | 4/2004  |
| JP A-2006-276060 | 10/2006 |
| JP A-2008-096539 | 4/2008  |
| JP A-2010-139643 | 6/2010  |

**OTHER PUBLICATIONS**

Apr. 18, 2013 Office Action issued in U.S. Appl. No. 13/235,041.  
Jan. 7, 2013 Office Action issued in U.S. Appl. No. 13/235,041.  
U.S. Appl. No. 13/235,041 to Fujita et al., filed Sep. 16, 2011.

\* cited by examiner

*Primary Examiner* — Stewart Fraser  
(74) *Attorney, Agent, or Firm* — Oliff PLC

(57) **ABSTRACT**

A toner for developing an electrostatic image, includes: colored particles containing a colorant and a binder resin, and two or more kinds of inorganic particles that are externally added to a surface of the colored particles, in which the two or more kinds of inorganic particles contain titanium-containing particles and silica-containing particles, an exposure ratio of the surface of the colored particles is about 25% or less, and a ratio of the titanium-containing particles that are in contact with the colored particles is about 15% by number or less.

**15 Claims, 3 Drawing Sheets**



FIG. 1



FIG. 2



FIG.3



## 1

**TONER FOR DEVELOPING  
ELECTROSTATIC IMAGE, METHOD OF  
PRODUCING TONER, CARTRIDGE, IMAGE  
FORMING METHOD, AND IMAGE FORMING  
APPARATUS**

**CROSS-REFERENCE TO RELATED  
APPLICATION**

This application is based on and claims priority under 35 USC 119 from Japanese Patent Application No. 2011-070899 filed Mar. 28, 2011.

**BACKGROUND**

1. Technical Field

The present invention relates to a toner for developing an electrostatic image, a method of producing the toner, a cartridge, an image forming method, and an image forming apparatus.

2. Related Art

A method of visualizing image information through an electrostatic latent image, for example, an electrophotographic process, is currently applied to various fields of art. In the electrophotographic process, an electrostatic latent image is formed on a surface of a photoconductor through charging and exposing, and the electrostatic latent image is developed with a developer containing a toner, and then visualized through transferring and fixing.

A dry developer is roughly classified into a single-component developer using a toner containing a colorant dispersed in a binder resin, and a two-component developer containing the toner and a carrier. Examples of the single-component developer include a magnetic single-component toner using a magnetic toner, and a non-magnetic single-component toner using a non-magnetic toner.

**SUMMARY**

According to an aspect of the invention, there is provided a toner for developing an electrostatic image, including: colored particles containing a colorant and a binder resin, and two or more kinds of inorganic particles that are externally added to a surface of the colored particles, wherein the two or more kinds of inorganic particles contain titanium-containing particles and silica-containing particles, an exposure ratio of the surface of the colored particles is about 25% or less, and a ratio of the titanium-containing particles that are in contact with the colored particles is about 15% by number or less.

**BRIEF DESCRIPTION OF THE DRAWINGS**

Exemplary embodiments of the present invention will be described in detail based on the following figures, wherein:

FIG. 1 is a schematic illustration showing a difference in an external addition state of silica-containing particles to colored particles depending on an adhesion method;

FIG. 2 is a schematic cross sectional view showing one example of an image forming apparatus using a two-component developer according to an exemplary embodiment; and

FIG. 3 is a schematic view showing one example of a developing device using a non-magnetic single-component developer according to an exemplary embodiment.

**DETAILED DESCRIPTION**

Exemplary embodiments of the invention are described in detail below.

## 2

**Toner for Developing Electrostatic Image**

A toner for developing an electrostatic image according to the exemplary embodiment includes: colored particles containing a colorant and a binder resin, and two or more kinds of inorganic particles that are externally added to a surface of the colored particles, in which the two or more kinds of inorganic particles contain titanium-containing particles and silica-containing particles, an exposure ratio of the surface of the colored particles is 25% or less, and a ratio of the titanium-containing particles that are in contact with the colored particles is 15% by number or less.

**Measurement Method of Exposure Ratio of Surface of Colored Particles**

The exposure ratio (E) of the surface of the colored particles in the exemplary embodiment may be obtained from a measured coverage of the silica-containing particles (Cs) on the surface of the colored particles and a measured coverage of the titanium-containing particles (Ct) on the surface of the colored particles. Specifically, the measured coverages Cs and Ct may be obtained by measuring the colored particles solely, the silica-containing particles solely, the titanium-containing solely, and the toner containing the silica-containing particles and the titanium-containing particles, for signal intensities of silicon atom and titanium atom respectively with an X-ray photoelectron spectroscopy (XPS) apparatus (JPS-9000MX, available from JEOL, Ltd.), and calculating according to the following expressions (1) and (2).

$$Ct = (Pt - Nt) / (Tt - Nt) \times 100(\%) \quad (1)$$

$$Cs = (Ps - Ns - Ct \times Ts) / (Ss - Ns) \times 100(\%) \quad (2)$$

Accordingly, the exposure ratio (E) may be calculated according to the following expression (3).

$$E = 100 - Ct - Cs(\%) \quad (3)$$

In the expressions (1) and (2), Ps represents the signal intensity of silicon atom derived from the silica-containing particles and the titanium-containing particles of the toner containing the silica-containing particles and the titanium-containing particles, Pt represents the signal intensity of titanium atom derived from the silica-containing particles and the titanium-containing particles of the toner, Ss represents the signal intensity of silicon atom of the silica-containing particles solely, Ts represents the signal intensity of silicon atom of the titanium-containing particles solely, Tt represents the signal intensity of titanium atom of the titanium-containing particles solely, Ns represents the signal intensity of silicon atom of the colored particles solely, and Nt represents the signal intensity of titanium atom of the colored particles solely.

**Measurement Method of Ratio of Titanium-Containing Particles that are in Direct Contact with Surface of Colored Particles**

In the exemplary embodiment, the ratio of the titanium-containing particles that are in direct contact with the surface of the colored particles (% by number) is obtained in the following manner. The language "the ratio of the titanium-containing particles that are in contact with the colored particles" means the ratio of the titanium-containing particles that are in direct contact with the surface of the colored particles.

A micrograph of the toner with a magnification of 30,000 is taken with a scanning electron microscope (FE-SEM S-4700, available from Hitachi, Ltd.) at an acceleration voltage of 5 kV. The number of the titanium-containing particles that are in contact with the colored particles is counted visually, and the ratio of the titanium-containing particles that are in con-

tact with the surface of the colored particles is calculated. In the exemplary embodiment, the ratios are calculated for 10 micrographs, and the average value thereof is designated as the ratio of the titanium-containing particles that are in contact with the surface of the colored particles.

In the determination as to whether or not a titanium-containing particle is in contact with a colored particle, it is determined that the titanium-containing particle is not in contact with the colored particle in the case where a silica-containing particle under the titanium-containing particle is visually observed around the titanium-containing particle, and it is determined that the titanium-containing particle is in contact with the colored particle in the case where a silica-containing particle under the titanium-containing particle is not visually observed around the titanium-containing particle.

#### External Additive

The toner for developing an electrostatic image of the exemplary embodiment has two or more kinds of inorganic particles that are externally added as an external additive to the surface of the colored particles, in which the two or more kinds of inorganic particles contain titanium-containing particles and silica-containing particles, the exposure ratio of the surface of the colored particles is 25% or less (or about 25% or less), and the ratio of the titanium-containing particles that are in contact with the surface of the colored particles is 15% by number or less (or about 15% by number or less).

In the toner for developing an electrostatic image of the exemplary embodiment, the exposure ratio of the surface of the colored particles is 25% or less, and the ratio of the titanium-containing particles that are in contact with the surface of the colored particles (which may be referred to as the contact ratio) is 15% by number or less, that is, the ratio of the titanium-containing particles that are in contact with the surface of the colored particles is lowered. Accordingly, it is expected that the titanium-containing particles may be prevented from being buried under the surface of the colored particles with thermal history and mechanical stress, thereby maintaining the charge exchangeability, and consequently the density stability of the image may be maintained. It is also expected that in the toner for developing an electrostatic image of the exemplary embodiment, the titanium-containing particles buried under the colored particles function as a filler to increase the melt viscosity on the surface of the colored particles, and the minimum fixing temperature may be prevented from being changed.

The toner for developing an electrostatic image of the exemplary embodiment may be preferably produced in such a manner that the silica-containing particles are firstly added to the surface of the colored particles without overlapping in the radial direction of the colored particles, and then the titanium-containing particles are externally added thereto. In the toner for developing an electrostatic image of the exemplary embodiment, the titanium-containing particles may be preferably added to the surface of the colored particles to form single layer without overlapping in the radial direction of the colored particles. When the titanium-containing particles are added to form single layer, it is expected that the amount of silica-containing particles positioned as an upper layer of the overlap is small, and thus the amount of the silica-containing particles that are released off is decreased, thereby preventing the silica-containing particles from being transferred to a carrier, a developer holding member, a photococonductor or the like. The addition in single layer may be confirmed directly by observation with an optical or electron microscope, or may be quantitatively confirmed by achieving the prescribed exposure ratio of the colored particles within the range of addition amount described later.

When the exposure ratio exceeds 25%, the surface of the colored particles is not sufficiently covered, and the frequency where the titanium-containing particles are in direct contact with the surface of the colored particles is increased, thereby failing to provide a contact ratio of the titanium-containing particles to the surface of the colored particles of 15% by number or less.

The exposure ratio of the surface of the colored particles may be preferably 23% or less, more preferably 20% or less, and still more preferably 16% or less (or about 16% or less). The lower limit of the exposure ratio of the surface of the colored particles is not particularly limited, and may be preferably 2% or more (or about 2% or more), and more preferably 3% or more, from the standpoint of production.

When the ratio of the titanium-containing particles that are in direct contact with the colored particles (contact ratio) is 15% by number or less, the titanium particles that are in direct contact with the colored particles may be prevented from being buried, whereby the charge exchangeability may be maintained, and the melt viscosity on the surface of the colored particles is increased, thereby suppressing the influence on the low temperature fixing property.

The ratio of the titanium-containing particles that are in direct contact with the colored particles (contact ratio) is preferably 12% by number or less, and more preferably 10% by number or less. The lower limit of the ratio of the titanium-containing particles that are indirect contact with the colored particles (contact ratio) is not particularly limited, and may be 0.5% by number or more, and preferably 1% by number or more, from the standpoint of production.

#### Silica-Containing Particles

The toner for developing an electrostatic image of the exemplary embodiment contains the two or more kinds of inorganic particles that are externally added as an external additive to the surface of the colored particles, and the two or more kinds of inorganic particles contain silica-containing particles.

The silica-containing particles are ordinarily used for enhancement of charging property and fluidity of a toner for developing an electrostatic image, and may be used from the standpoint of cost.

The toner for developing an electrostatic image of the exemplary embodiment has an exposure ratio of the surface of the colored particles of 25% or less, and a ratio of the titanium-containing particles that are in contact with the colored particles is 15% by number or less, and the toner may preferably have at least single layer formed with the silica-containing particles added in an amount that is larger than the titanium-containing particles, on the surface of the colored particles. The layer formed with the silica-containing particles added to the surface of the colored particles may not cover the entire surface of the colored particles but provides an exposure ratio on the surface of the colored particles of 25% or less. Accordingly, there may be a portion where the surface of the colored particles is exposed is present among the silica-containing particles added to the surface of the colored particles, and the surface of the colored particles may have a portion where no silica-containing particle is added and a portion where the titanium-containing particles are added.

The silica-containing particles may have a volume average particle diameter of from 5 nm to 40 nm (or from about 5 nm to about 40 nm), and preferably from 7 nm to 30 nm. When the volume average particle diameter of the silica-containing particles is 5 nm or more, the adhesion property to the surface of the colored particles may be favorably enhanced, and the silica-containing particles are conveniently produced. When

the volume average particle diameter is 40 nm or less, the charging property and the fluidity may be favorably enhanced, and the silica-containing particles may be suitable for a non-magnetic single-component toner, which is demanded to have charging property and fluidity. Furthermore, the addition amount of the silica-containing particles that is required for covering the surface of the colored particles with single layer may be small, which is favorable from the standpoint of cost.

Examples of the production method of the silica-containing particles include a vapor phase production method, a wet production method, a sol-gel production method and the like, and the silica-containing particles that are produced by a vapor phase production method may be used since the silica-containing particles having a small particle diameter may be produced at low cost.

The silica-containing particles may be subjected to a surface treatment, for example, may be subjected to a surface treatment for imparting hydrophobicity with a silane coupling agent, a titanium coupling agent, a silicone oil or the like. The silica-containing particles having a hydrophobic surface has low affinity to the surface of the colored particle, which prevents the silica-containing particles from being buried under the surface. The material used for the surface treatment may be a silane coupling agent, which may provide favorable charging property and fluidity.

The amount of the silica-containing particles added may be such an amount that provides a coverage on the colored particles of from 90% to 150%. When the coverage is 90% or more, the intended exposure ratio may be obtained by providing single layer containing the silica-containing particles added without overlapping in the radial direction of the colored particles. When the coverage is 150% or less, a less amount of the silica-containing particles occur that remain after adding as single layer on the surface of the colored particles, and the probability of occurrence of two or more layers added to the surface of the colored particles may be favorably decreased.

The amount of the silica-containing particles added may be preferably such an amount that provides a coverage on the colored particles of from 95% to 135%.

The coverage of the silica-containing particles on the toner particles may be obtained according to the following expression.

$$\text{coverage}(\%) = (\sqrt{3}/(2\pi)) \times (dt/da) \times (\rho_t/\rho_a) \times C \times 100$$

wherein

da: the weight average particle diameter of the external additive (silica-containing particles),

dt: the weight average particle diameter of the toner particles,

$\rho_a$ : the true specific gravity of the external additive,

$\rho_t$ : the true specific gravity of the toner particles,

C: the ratio (weight of external additive)/(weight of toner particles)

#### Titanium-Containing Particles

The toner for developing an electrostatic image of the exemplary embodiment contains the two or more kinds of inorganic particles that are externally added as an external additive to the surface of the colored particles, and the two or more kinds of inorganic particles contain titanium-containing particles.

In general, the titanium-containing particles facilitate the charge exchangeability among toner particles to improve the charge distribution, but, owing to the high affinity thereof to a resin as compared to the silica-containing particles, are liable to be buried under the surface of the colored particles through

storage under heat, and mechanical stress. In particular, the titanium-containing particles have high affinity to a polyester resin, and may be notably buried under the colored particles in the case where a polyester resin is used as the binder resin.

When the titanium-containing particles are buried under the colored particles, the charge exchangeability may be lowered, which broadens the charge distribution. Furthermore, the titanium-containing particles may function as a filler, which increases the melt viscosity on the surface of the colored particle, thereby deteriorating the low temperature fixing property.

In the exemplary embodiment of the invention, it is preferred that the silica-containing particles are firstly added to the surface of the colored particles without overlapping in the radial direction of the colored particles, and then the titanium-containing particles are externally added thereto. It is thought that the charge exchangeability is increased by externally adding the titanium-containing particles to the colored particles, and the charge distribution is narrowed. It is also thought that the exemplary embodiment of the invention may effective for the improvement of the fluidity.

The toner for developing an electrostatic image of the exemplary embodiment has an exposure ratio of the surface of the colored particles of 25% or less and a ratio of the titanium-containing particles that are in contact with the surface of the colored particles of 15% by number or less, and thus 85% by number of the titanium-containing particles are not in direct contact with the colored particles but are present on the silica-containing particles that are added directly to the surface of the colored particles. In the toner for developing an electrostatic image of the exemplary embodiment, 85% by number of the titanium-containing particles may be present on a layer formed with the silica-containing particles added directly to the surface of the colored particles.

Examples of the titanium-containing particles include anatase type titanium oxide particles, rutile type titanium oxide particles and metatitanic acid particles. Even rutile type titanium oxide particles, which are ordinarily liable to be buried under the colored particles, among these may be used in the exemplary embodiment.

The titanium-containing particles may have a volume average particle diameter of from 8 nm to 50=(or from about 8 nm to about 50 nm), and preferably from 10 nm to 40 nm. When the volume average particle diameter of the titanium-containing particles is 8 nm or more, the particles may have good dispersibility, which facilitates adhesion in the form of primary particles. When the volume average particle diameter is 50 nm or less, the particles may be prevented from being released from the toner, and good fluidity may be obtained.

The volume average particle diameter of the titanium-containing particles may be larger than the volume average particle diameter of the silica-containing particles. The volume average particle diameter of the titanium-containing particles that is larger than the volume average particle diameter of the silica-containing particles may decrease the probability of adhesion of the titanium-containing particles to the surface of the colored particles through among the silica-containing particles added to the surface of the colored particles.

The amount of the titanium-containing particles added may be such an amount that provides a coverage on the colored particles of from 10% to 50%, and preferably from 15% to 45%. When the amount provides a coverage of 10% or more, sufficient charge exchangeability may be obtained. When the amount provides a coverage of 50% or less, the particles may be prevented from being released from the

toner. The coverage of the titanium-containing particles may be calculated in the same manner as in the coverage of the silica-containing particles.

The total of a coverage of the titanium-containing particles and a coverage of the silica-containing particles may be 150% or less.

The ratio of coverage of the titanium-containing particles to the silica-containing particles may be from 1/2 to 1/10 based on the addition amounts.

The toner for developing an electrostatic image of the exemplary embodiment may contain an additional external additive in such an amount that does not impair the advantages of the exemplary embodiment, and may contain only the titanium-containing particles and the silica-containing particles as an external additive.

Examples of the additional external additive include inorganic particles, such as alumina and cerium oxide, and organic particles, such as polymethyl methacrylate (PMMA) particles.

#### Colored Particles

The colored particles in the toner for developing an electrostatic image of the exemplary embodiment contain at least a colorant and a binder resin.

The colored particles may further contain, in addition to these components, other components, such as a release agent.

#### Binder Resin

The binder resin in the exemplary embodiment is not particularly limited, and known resins for colored particles may be used. For example, from the standpoint of low temperature fixing property, a polyester resin may be used and an amorphous (non-crystalline) polyester resin may be used preferably. The polyester resin may be synthesized, for example, through polycondensation of mainly a polyvalent carboxylic acid and a polyol.

The amorphous polyester resin referred herein means a resin that exhibits stepwise endothermic change without clear peaks in differential scanning calorimetry (which may be hereinafter abbreviated as DSC).

#### Colorant

The colored particles contain a colorant.

The colorant may be either a dye or a pigment, and may be a pigment from the standpoint of light resistance and water resistance. The colorant is not limited to a chromatic colorant and may be a white colorant and a colorant exhibiting metallic color.

Examples of the colorant include known pigments, such as carbon black, Aniline Black, Aniline Blue, Calco Oil Blue, Chrome Yellow, Ultramarine Blue, Du Pont Oil Red, Quinoline Yellow, Methylene Blue Chloride, Phthalocyanine Blue, Malachite Green Oxalate, lamp black, Rose Bengal, quinacridone, Benzidine Yellow, C.I. Pigment Red 48:1, C.I. Pigment Red 57:1, C.I. Pigment Red 122, C.I. Pigment Red 185, C.I. Pigment Red 238, C.I. Pigment Yellow 12, C.I. Pigment Yellow 17, C.I. Pigment Yellow 180, C.I. Pigment Yellow 97, C.I. Pigment Yellow 74, C.I. Pigment Blue 15:1 and C.I. Pigment Blue 15:3.

In the exemplary embodiment, the content of the colorant in the toner for developing an electrostatic image may be in a range of from 1 part by weight to 30 parts by weight per 100 parts by weight of the binder resin.

A colorant having been subjected to a surface treatment may be used, and a pigment dispersant may be used. A colored toner, such as a yellow toner, a magenta toner, a cyan toner and a black toner, may be obtained by selecting the kind of the colorants.

#### Release Agent

The colored particles may contain a release agent.

Examples of the release agent include paraffin wax, such as low molecular weight polypropylene and low molecular weight polyethylene, a silicone resin, a rosin compound, rice wax, and carnauba wax.

The release agent may have a melting temperature of from 50° C. to 100° C., and preferably from 60° C. to 95° C.

The content of the release agent in the colored particles may be from 0.5% to 15% by weight, and preferably from 1.0% to 12% by weight. When the content of the release agent is 0.5% by weight or more, releasing failure may be prevented from occurring particularly in oil-less fixing. When the content of the release agent is 15% by weight or less, the fluidity of the toner may be prevented from being deteriorated, thereby ensuring the image quality and the reliability of image formation.

#### Other Additives

The colored particles may contain, in addition to the aforementioned components, various components, such as an internal additive and a charge controlling agent.

Examples of the internal additive include a magnetic material, for example, ferrite, magnetite, a metal, such as reduced iron, cobalt, nickel and manganese, alloys of these metals, and compounds of these metals.

Examples of the charge controlling agent include a quaternary ammonium salt compound, a nigrisine compound, a dye containing a complex of aluminum, iron, chromium or the like, and a triphenylmethane pigment.

#### Characteristics of Toner

The toner for developing an electrostatic image of the exemplary embodiment may have a degree of circularity of from 0.950 to 0.980, and preferably from 0.958 to 0.976.

The degree of circularity may be obtained through image analysis, and may be measured, for example, with FPIA-3000 (available from Sysmex Corporation).

The toner for developing an electrostatic image of the exemplary embodiment may have a volume average particle diameter of from 3 μm to 9 μm, preferably from 3.1 μm to 8.5 μm, and more preferably from 3.2 μm to 8.0 μm. When the volume average particle diameter is 3 μm or more, the fluidity may be prevented from being lowered, and the charging property may be maintained. When the volume average particle diameter is 9 μm or less, the resolution may be prevented from being decreased. The volume average particle diameter may be measured with such a measuring apparatus as Coulter Multisizer II (available from Beckman Coulter, Inc.).

#### Production Method of Toner for Developing Electrostatic Image

The production method of the toner for developing an electrostatic image of the exemplary embodiment is not particularly limited as long as the method provides the toner meeting the above requirements, and such a method may be employed that contains, for example, preparation of the colored particles containing a colorant and a binder resin (which may be hereinafter referred to as preparation of colored particles), addition of the silica-containing particles to the colored particles in an aqueous medium, through wet external addition to provide the colored particles having the silica-containing particles added (which may be hereinafter referred to as addition of silica-containing particles), and addition of the titanium-containing particles to the colored particles having the silica-containing particles added, through dry external addition (which may be hereinafter referred to as addition of titanium-containing particles).

60  
65

## Preparation of Colored Particles

The production method of the toner for developing an electrostatic image of the exemplary embodiment may contain the preparation of the colored particles containing a colorant and a binder resin (preparation of colored particles).

The preparation method of the colored particles in the preparation of the colored particles is not particularly limited, and examples of the preparation method include known methods, for example, a dry method, such as a kneading and pulverizing method, a wet method, such as a melting and suspension method, an emulsification and aggregation method and a dissolution and suspension method.

## Addition of Silica-Containing Particles

The production method of the toner for developing an electrostatic image of the exemplary embodiment may contain the addition of the silica-containing particles to the colored particles in an aqueous medium, through wet external addition to provide the colored particles having the silica-containing particles added (addition of silica-containing particles).

In the wet external addition, the silica-containing particles are added without overlapping in the radial direction of the colored particles irrespective of the shape of the colored particles. Accordingly, the added state in single layer of the silica-containing particles is realized, which is not easily achieved by dry external addition.

The addition of silica-containing particles may include, for example, addition of silica-containing particles to the surface of the colored particles in an aqueous medium by adding the silica-containing particles to the dispersion liquid of the colored particles, and drying of the resulting colored particles having the silica-containing particles added.

Examples of the aqueous medium used in the exemplary embodiment include water, such as distilled water and ion exchanged water, and an alcohol, such as ethanol and methanol. Among these, ethanol and water are preferred, and water, such as distilled water and ion exchanged water, is more preferred. The aqueous medium may be used solely or as a combination of two or more kinds thereof.

The aqueous medium may contain a water miscible organic solvent. Examples of the water miscible organic solvent include acetone and acetic acid.

The dispersion liquid of the colored particles in the addition of silica-containing particles may have a solid content ratio of 20% or more, and preferably 25% or more. When the solid content ratio is 20% or more, it is considered that the silica-containing particles are added without overlapping in the radial direction of the colored particles through a hetero-aggregation mechanism. The solid content ratio may be 50% or less, and preferably 45% or less. When the solid content ratio is 50% or less, positional heterogeneity in stirring in the dispersion liquid may be suppressed.

As a method of adding the silica-containing particles to the dispersion liquid of the colored particles, the silica-containing particles in a solid state (i.e., in the form of powder) may be added directly to the dispersion liquid of the colored particles, or a dispersion liquid having the silica-containing particles dispersed therein may be added to the dispersion liquid of the colored particles. The silica-containing particles that have been subjected to a hydrophobic treatment are hard to be dispersed in the aqueous medium, and therefore, the silica-containing particles having been dispersed in a mixed solvent of methanol and water in advance may be added to the dispersion liquid of the colored particles. The mixing ratio of methanol and water (methanol/water) in the mixed solvent may be from 1/9 to 5/5.

In the addition of silica-containing particles, the silica-containing particles may be added to the colored particles by making the pH of the dispersion liquid of the colored particles having the silica-containing particles added thereto acidic under stirring of the dispersion liquid. The range of the pH may be in a range of from 2 to 6.5, and preferably from 3 to 6. When the pH is 6.5 or less, dissociation of a carboxylic acid and the like on the surface of the colored particles is prevented from occurring, and thereby the silica-containing particles may be added without overlapping in the radial direction of the colored particles.

FIG. 1 is a schematic illustration showing the difference in the external addition state of the silica-containing particles to the colored particles depending on the adhesion method. The states (c) and (d) may be employed in the exemplary embodiment, and the state (c) may be preferred.

The state (a) in FIG. 1 schematically shows an example where the silica-containing particles in an amount corresponding to a coverage of 100% are added to the colored particles by dry external addition.

In the state (a) in FIG. 1, it is observed that the silica-containing particles form aggregates  $P_c$  and are externally added in the form of aggregates  $P_c$  to the colored particles, and the surface of the colored particles is exposed frequently. Furthermore, it is also observed that the silica-containing particles partly form free particles  $P_i$ .

The state (b) in FIG. 1 schematically shows an example where the silica-containing particles in an amount corresponding to a coverage of 150% are added to the colored particles by dry external addition.

In the state (b) in FIG. 1, as similar to the state (a) in FIG. 1, it is observed that the silica-containing particles form aggregates  $P_c$  and are externally added in the form of aggregates  $P_c$  to the colored particles, and the surface of the colored particles is exposed frequently. Furthermore, it is also observed that the silica-containing particles partly form free particles  $P_i$ .

The state (c) in FIG. 1 schematically shows an example where the silica-containing particles in an amount corresponding to a coverage of 100% are added to the colored particles by wet external addition.

In the state (c) in FIG. 1, it is observed that the silica-containing particles do not form aggregates  $P_c$  and are externally added in the form of single layer on the colored particles, and the surface of the colored particles is substantially not exposed. Furthermore, it is also observed that the silica-containing particles substantially do not form free particles  $P_i$ .

The state (d) in FIG. 1 schematically shows an example where the silica-containing particles in an amount corresponding to a coverage of 150% are added to the colored particles by wet external addition.

In the state (d) in FIG. 1, it is observed that the silica-containing particles do not form aggregates  $P_c$  and are externally added in the form of one or more layers on the colored particles, and the surface of the colored particles is substantially not exposed. Furthermore, it is also observed that the silica-containing particles are partly on top of others and free particles  $P_i$ .

The colored particles having been subjected to the addition of silica-containing particles are subjected to solid-liquid separation by filtration and then subjected to the drying by vacuum freeze drying, thereby providing the colored particles having the silica-containing particles added thereto. The colored particles having the silica-containing particles added thereto may be subjected to rinsing where the colored particles are rinsed before the drying.

## 11

## Addition of Titanium-Containing Particles

The production method of the toner for developing an electrostatic image of the exemplary embodiment may contain the addition of the titanium-containing particles to the colored particles having the silica-containing particles added thereto, through dry external addition (addition of titanium-containing particles).

In the addition of titanium-containing particles, examples of the method of externally adding the titanium-containing particles to the surface of the colored particles having the silica-containing particles uniformly added thereto include a known dry external addition method. Examples of a mixer used in the dry external addition method include known mixers, such as a V-blender, a Henschel mixer and a Loedige mixer.

By the dry external addition of the titanium particles to the colored particles having the silica particles added, the titanium particles are externally added onto the layer of the silica particles, and thus the probability of contact of the titanium-containing particles to the surface of the colored particles is decreased, thereby providing the toner having a contact ratio of the titanium-containing particles to the surface of the colored particles of 15% by number or less.

Another external additive may be added along with the addition of silica-containing particles and the addition of titanium-containing particles.

## Developer for Developing Electrostatic Image

The toner for developing an electrostatic image of the exemplary embodiment may be used as a non-magnetic single-component developer or a two-component developer. In the case where the toner is used as a two-component developer, the toner may be mixed with a carrier.

The carrier used in the two-component developer is not particularly limited, and known carriers may be used. Examples of the carrier include iron oxide, a magnetic metal, such as nickel and cobalt, a magnetic oxide, such as ferrite and magnetite, a resin coated carrier having a resin coating layer on these materials as a core, a magnetic material dispersed carrier, and a resin dispersed carrier which contains electroconductive material dispersed in a matrix resin.

Examples of the coating resin and the matrix resin used for the carrier include polyethylene, polypropylene, polystyrene, polyvinyl acetate, polyvinyl alcohol, polyvinyl butyral, polyvinyl chloride, polyvinyl ether, polyvinyl ketone, a vinyl chloride-vinyl acetate copolymer, a styrene-acrylic acid copolymer, a linear silicone resin containing organosiloxane bonds and a modified product thereof, a fluorine resin, polyester, polycarbonate, a phenol resin and an epoxy resin, but the resins are not limited to these examples.

Examples of the electroconductive material include a metal, such as gold, silver and copper, carbon black, titanium oxide, zinc oxide, barium sulfate, aluminum borate, potassium titanate, tin oxide and carbon black, but the electroconductive material is not limited to these examples.

Examples of the core material of the carrier include a magnetic metal, such as iron, nickel and cobalt, a magnetic oxide, such as ferrite and magnetite, and glass beads, and a magnetic material may be used when the carrier is applied to a magnetic brush system. The volume average particle diameter of the core material of the carrier may be in a range of from 10  $\mu\text{m}$  to 500  $\mu\text{m}$ , and preferably from 30  $\mu\text{m}$  to 100  $\mu\text{m}$ .

Examples of the method for coating the resin on the surface of the core material of the carrier include a method of coating a solution for forming the resin coating layer, which contains the coating resin and other additives depending on necessity, dissolved in an appropriate solvent. The solvent is not par-

## 12

ticularly limited, and may be selected in consideration of the coating resin used, the coating suitability and the like.

Specific examples of the method of coating the resin include a dipping method of dipping the core material of the carrier in the solution for forming the coating layer, a spraying method of spraying the solution for forming the coating layer onto the surface of the core material of the carrier, a fluidized bed method of spraying the solution for forming the coating layer onto the surface of the core material of the carrier that is in a fluidized state with fluidizing air, and a kneader-coater method of mixing the core material of the carrier and the solution for forming the coating layer in a kneader-coater, followed by removing the solvent.

The mixing ratio (by weight) of the toner for developing an electrostatic image of the exemplary embodiment and the carrier in the two-component developer may be a toner/carrier ratio of from 1/100 to 30/100, and preferably from 3/100 to 20/100.

## 20 Cartridge, Image Forming Method and Image Forming Apparatus

The cartridge according to the exemplary embodiment is described below.

The cartridge of the exemplary embodiment may accommodate at least the toner for developing an electrostatic image of the exemplary embodiment or the developer for developing an electrostatic image of the exemplary embodiment. The cartridge of the exemplary embodiment may be detachable from an image forming apparatus.

30 In the case where the cartridge is applied to an image forming method or an image forming apparatus, the cartridge may be a toner cartridge accommodating the toner of the exemplary embodiment solely, a developer cartridge accommodating the developer of the exemplary embodiment, or a process cartridge containing a developing unit that forms a toner image through development of an electrostatic latent image formed on an image holding member, with the toner for developing an electrostatic image of the exemplary embodiment or the developer for developing an electrostatic image of the exemplary embodiment.

The process cartridge of the exemplary embodiment may further contain other members, such as an erasing unit, depending on necessity.

45 The image forming method of the exemplary embodiment may contain: latent image formation of forming an electrostatic latent image on a surface of an image holding member; development of developing the electrostatic latent image formed on the surface of the image holding member, with a toner, to form a toner image; transferring the toner image formed on the surface of the image holding member, to a surface of a transfer medium; and fixing the toner image transferred to the surface of the transfer medium, in which the toner may be the toner for developing an electrostatic image 50 of the exemplary embodiment.

The toner may be the toner for developing an electrostatic image of the exemplary embodiment or a two-component developer containing the toner for developing an electrostatic image of the exemplary embodiment and a carrier.

60 In the image forming method of the exemplary embodiment, a developer containing the toner for developing an electrostatic image of the exemplary embodiment may be prepared, an electrostatic image may be formed and developed with the developer in an ordinary electrophotographic copying machine, and the resulting toner image may be transferred electrostatically to transfer sheet and fixed thereto with a fixing device, to form a copied image.

The image forming method of the exemplary embodiment may employ a non-magnetic single-component developer system.

The aforementioned processes are each an ordinary process, and are described, for example, in JP-A-56-40868, JP-A-49-91231 and the like. The image forming method of the exemplary embodiment may be practiced with a known image forming apparatus, such as a copying machine and a facsimile machine.

The formation of an electrostatic latent image is a process of forming an electrostatic latent image on an image holding member (photoconductor).

The development is a process of developing the electrostatic latent image with a developer layer on a developer holding member, thereby forming a toner image. The developer layer is not particularly limited as far as it contains the toner for developing an electrostatic image of the exemplary embodiment.

The transferring is a process of transferring the toner image to a transfer medium. Examples of the transfer medium in the transferring include an intermediate transfer medium and a recording medium, such as paper.

In the fixing, the toner image transferred on the transfer paper is fixed with a heating roller fixing device having a heating roller with a temperature controlled to a prescribed value, and thereby a copied image is formed.

The image forming method of the exemplary embodiment may contain cleaning. The cleaning is a process of removing the developer for developing an electrostatic image remaining on the image holding member.

The recording medium used may be a known one. Examples of the recording medium include paper and an OHP sheet, which are used in a copying machine, a printer or the like of an electrophotographic system, and coated paper obtained by coating ordinary paper with a resin or the like on the surface thereof, art paper for printing, and the like may be used.

The image forming method of the exemplary embodiment may further contain recycling. The recycling is a process step of moving the toner for developing an electrostatic image thus collected in the cleaning, to the developer layer. The image forming method of the exemplary embodiment that contains the recycling may be practiced with an image forming apparatus, such as a copying machine and a facsimile machine, with a toner recycling system. The image forming method may also be applied to a recycling system, in which the toner is collected simultaneously with the development without cleaning.

The image forming apparatus of the exemplary embodiment may contain: an image holding member; a charging unit that charges the image holding member; an exposing unit that exposes the charged image holding member, to form an electrostatic latent image on the image holding member; a developing unit that develops the electrostatic latent image with a toner, to form a toner image; a transferring unit that transfers the toner image from the image holding member to a transfer medium; and a fixing unit that fixes the toner image transferred to the surface of the transfer medium, in which the toner may be the toner for developing an electrostatic image of the exemplary embodiment.

The image forming apparatus of the exemplary embodiment is not particularly limited as far as the image forming apparatus contains at least the image holding member, the charging unit, the exposing unit, the developing unit, the transferring unit and the fixing unit, and may further contain a cleaning unit, an erasing unit and the like depending on necessity.

In the transferring unit, the transferring operation may be performed twice or more by using an intermediate transfer medium. Examples of the transfer medium in the transferring include an intermediate transfer medium and a recording medium, such as paper.

In the image holding member and the units of the image forming apparatus of the exemplary embodiment, the constitutions described for the processes of the image forming method of the exemplary embodiment may be preferably employed. The units may employ the well known units for the image forming apparatus. The image forming apparatus of the exemplary embodiment may further contain other units and devices than the units and devices described above. In the image forming apparatus of the exemplary embodiment, plural units among the units described may be performed simultaneously.

An example of the image forming apparatus of the exemplary embodiment is described with reference to FIG. 2, but the exemplary embodiment is not limited to the example. FIG. 2 is a schematic cross sectional view showing the example of the image forming apparatus using a two-component developer according to the exemplary embodiment.

FIG. 2 is a schematic illustration showing an example of a structure of an image forming apparatus for forming an age 25 according to the image forming method of the exemplary embodiment. The image forming apparatus 200 shown in the figure has inside a housing 400 four electrophotographic photoconductors (image holding members) 401a to 401d disposed in series along an intermediate transfer belt 409. The 30 electrophotographic photoconductors 401a to 401d are capable of forming color images, i.e., a yellow image is formed with the electrophotographic photoconductor 401a, a magenta image is formed with the electrophotographic photoconductor 401b, a cyan image is formed with the electrophotographic photoconductor 401c, and a black image is formed with the electrophotographic photoconductor 401d.

The electrophotographic photoconductors 401a to 401d are each rotatable in a prescribed direction (in the counter-clockwise direction in the figure), and charging rolls 402a to 402d, developing devices 404a to 404d, primary transfer rolls 410a to 410d, and cleaning blades 415a to 415d are disposed around the electrophotographic photoconductors 401a to 401d, respectively, along the rotation direction thereof. The developing devices 404a to 404d are capable of supplying toners of four colors, yellow, magenta, cyan and black, accommodated in the toner cartridges 405a to 405d, respectively, and the primary transfer rolls 410a to 410d are in contact with the electrophotographic photoconductors 401a to 401d, respectively, through the intermediate transfer belt 409.

An exposing device 403 is disposed at a prescribed position inside the housing 400 and is capable of radiating a light beam emitted from the exposing device 403 onto the surfaces of the electrophotographic photoconductors 401a to 401d after 55 charging. According to the structure, the processes of charging, exposing, developing, primary transferring and cleaning are performed in the rotation process of each of the electrophotographic photoconductors 401a to 401d, and thereby toner images of the colors are transferred and layered on the intermediate transfer belt 409.

The charging rolls 402a to 402d apply a voltage to the electrophotographic photoconductors 401a to 401d, respectively, to charge the surfaces of the photoconductors to a prescribed potential by bringing an electroconductive member (the charging roll) into contact with the surface of the electrophotographic photoconductor (i.e., the charging). In the exemplary embodiment, a charging brush, a charging

## 15

film, a charging tube or the like may be used instead of the charging roll, and a non-contact charging system using corotron or scorotron may also be used.

The exposing device 403 may be, for example, an optical device capable of exposing imagewise the surfaces of the electrophotographic photoconductors 401a to 401d with a semiconductor laser, LED (light emitting diode), a liquid crystal shutter or the like as a light source.

In the developing devices 404a to 404d, developing may be performed with an ordinary developing device by contact or non-contact development with the two-component developer for developing an electrostatic image (i.e., the development). The developing device is not particularly limited as far as the developing device uses a two-component developer for developing an electrostatic image, and may be selected from known devices depending on purposes. In the primary transferring, the primary transfer rolls 410a to 410d are each applied with a primary transfer bias having a reverse polarity to the toners on the image holding members, and thereby the toners of the colors are primarily transferred sequentially from the image holding members to the intermediate transfer belt 409.

The cleaning blades 415a to 415d each remove the remaining toner added to the surface of the electrophotographic photoconductor after the transferring, and the electrophotographic photoconductor having the surface thus cleaned therewith is then used repeatedly for the next image formation process. Examples of the material of the cleaning blade include urethane rubber, neoprene rubber and silicone rubber.

The intermediate transfer belt 409 is supported under predetermined tension with a driving roll 406, a backup roll 408 and a tension roll 407, and is rotatable through rotation of the rolls without slack. A secondary transfer roll 413 is disposed to be in contact with the backup roll 408 through the intermediate transfer belt 409.

The secondary transfer roll 413 is applied with a secondary transfer bias having a reverse polarity to the toners on the intermediate transfer belt, and thereby the toners are secondarily transferred from the intermediate transfer belt to the recording medium. The surface of the intermediate transfer medium 409 passing through between the backup roll 408 and the secondary transfer roll 413 is then cleaned, for example, with a cleaning blade 416 disposed in the vicinity of the driving roll 406 or an erasing device (which is not shown in the figure), and the intermediate transfer belt is then used repeatedly for the next image formation process. A tray (recording medium tray) 411 is disposed at a prescribed position inside the housing 400, and the recording medium 500, such as paper, in the tray 411 is conveyed with a conveying roll 412 to between the intermediate transfer belt 409 and the secondary transfer roll 413 and then between two fixing rolls 414 in contact with each other, and then delivered outside the housing 400.

An example of an image forming apparatus, in which development is performed with a non-magnetic single-component developer, is described with reference to FIGS. 2 and 3. The image formation may be performed similarly by using a developing device 10 shown in FIG. 3 as each of the developing devices 404a to 404d in FIG. 2.

The toner for developing an electrostatic image of the exemplary embodiment may be preferably applied to a non-magnetic single-component developer. The reason is as follows in the non-magnetic single-component developer system, the surface of the toner receives larger stress, and the silica-containing particles added as an external additive are liable to be buried under the toner, as compared to the two-component developer system. However, it is considered that

## 16

the use of the toner for developing an electrostatic image of the exemplary embodiment may prevent the silica-containing particles from being buried under the toner even in the non-magnetic single-component developer system.

The developing device 10 shown in FIG. 3 contains: a developing roll 12 that is disposed in contact with a image holding member (photoconductor) 26, which is rotatable in the direction shown by the arrow A with a driving power source not shown in the figure, and is capable being driven and rotated in the direction shown by the arrow B with the rotation of the image holding member 26; a bias power source 14 that is connected to the developing roll 12; a toner scraping member 16 that is disposed in contact with the developing roll 12 under pressure at the position on the downstream side of the position where the developing roll 12 and the image holding member 26 are in contact with each other in the rotation direction of the developing roll 12, and is rotatable in the direction shown by the arrow C opposite to the rotation of the developing roll 12; a toner layer control member 18 that is disposed at the position on the downstream side of the position where the developing roll 12 and the toner scraping member 16 are in contact with each other under pressure and on the upstream side of the position where the developing roll 12 and the image holding member 26 are in contact with each other in the rotation direction of the developing roll 12, and is disposed in contact with the developing roll 12; a housing 22 that is disposed on the side of the developing roll 12 opposite to the side where the image holding member 26 is disposed, and has an opening on the side where the developing roll 12 is disposed; and an agitator 20 disposed inside the housing 22.

The toner layer control member 18 is fixed at one end thereof to the opening of the housing 22, thereby closing the opening of the housing 22. The opening of the housing 22 on the side (i.e., the lower side of the opening) opposite to the side where the toner layer control member 18 is provided (i.e., the upper side of the opening) is provided to cover the lower side of the developing roll 12 and the toner scraping member 16. The toner (i.e., the non-magnetic single-component developer) 24 is disposed as being accumulated on the lower side of the housing 22, and is accumulated in such a manner that the toner is filled in the space between the lower side of the developing roll 12 and the lower side of the opening of the housing 22 with no space and covers the toner scraping member 16. The toner 24 is fed with the agitator 20 provided inside the housing 22 from the interior of the housing 22 to the side of the opening of the housing 22 where the developing roll 12 is provided.

Upon development, the toner 24 in the housing 22 is fed to the surface of the developing roll 12 with the agitator 20 and the toner scraping member 16. The toner 24 added to the surface of the developing roll 12 is then added to form a toner layer having a uniform thickness on the surface of the developing roll 12 with the toner layer control member 18. Subsequently, the toner 24 added to the surface of the developing roll 12 is transferred to the image holding member 26 having an electrostatic latent image (which is not shown in the figure) formed thereon through the difference in potential between the surface of the image holding member 26 and the developing roll 12, which is applied with a bias voltage from a bias power source 14, thereby developing the electrostatic latent image. The toner 24 remaining on the surface of the developing roll 12 after completing the development is scraped off with the toner scraping member 16.

## EXAMPLES

The exemplary embodiments are described in more detail with reference to examples and comparative examples below,

but the invention is not limited to the examples. All the terms "part" and "%" in the following description indicate "part by weight" and "% by weight", respectively, unless otherwise indicated.

Measurement Method of Exposure Ratio of Surface of Colored Particles

The exposure ratio (E) of the surface of the colored particles is obtained from a measured coverage of the silica-containing particles (Cs) on the surface of the colored particles and a measured coverage of the titanium-containing particles (Ct) on the surface of the colored particles. Specifically, the measured coverages Cs and Ct are obtained by measuring the colored particles solely, the silica-containing particles solely, the titanium-containing particles solely, and the toner containing the silica-containing particles and the titanium-containing particles, for signal intensities of silicon atom and titanium atom respectively with an X-ray photo-electron spectroscopy (XPS) apparatus (JPS-9000MX, available from JEOL, Ltd.), and calculating according to the following expressions (1) and (2).

$$Ct = (Pt - Nt) / (Tt - Nt) \times 100 (\%) \quad (1)$$

$$Cs = (Ps - Ns - Ct \times Ts) / (Ss - Ns) \times 100 (\%) \quad (2)$$

Accordingly, the exposure ratio (E) is calculated according to the following expression (3).

$$E = 100 - Ct - Cs (\%) \quad (3)$$

In the expressions (1) and (2), Ps represents the signal intensity of silicon atom derived from the silica-containing particles and the titanium-containing particles of the toner containing the silica-containing particles and the titanium-containing particles, Pt represents the signal intensity of titanium atom derived from the silica-containing particles and the titanium-containing particles of the toner, Ss represents the signal intensity of silicon atom of the silica-containing particles solely, Ts represents the signal intensity of silicon atom of the titanium-containing particles solely, Tt represents the signal intensity of titanium atom of the titanium-containing particles solely, Ns represents the signal intensity of silicon atom of the colored particles solely, and Nt represents the signal intensity of titanium atom of the colored particles solely.

Measurement Method of Ratio of Titanium-Containing Particles that are in Contact with Surface of Colored Particles

A micrograph of the toner with a magnification of 30,000 is taken with a scanning electron microscope (FE-SEM S-4700, available from Hitachi, Ltd.). The number of the titanium-containing particles that are in contact with the colored particles is counted visually, and the ratio of the titanium-containing particles that are in contact with the surface of the colored particles is calculated. In the example, 10 micrographs of the toner are measured, and the average value thereof is designated as the ratio of the titanium-containing particles that are in contact with the surface of the colored particles (% by number).

In the visual determination as to whether or not a titanium-containing particle is in contact with a colored particle, it is determined that the titanium-containing particle is not in contact with the colored particle in the case where a silica-containing particle under the titanium-containing particle is visually observed around the titanium-containing particle, and it is determined that the titanium-containing particle is in contact with the colored particle in the case where a silica-containing particle under the titanium-containing particle is not visually observed around the titanium-containing particle.

1. Synthesis of Amorphous Polyester Resin (1)

90 parts by mol of polyoxyethylene(2,0)-2,2-bis(4-hydroxyphenyl)propane, 10 parts by mol of ethylene glycol, 80 parts by mol of terephthalic acid and 20 parts by mol of isophthalic acid as raw materials and dibutyltin oxide as a catalyst are put into a two-neck flask having been dried by heating, and the content of the flask is heated while maintaining the interior of the flask inert by introducing nitrogen gas. The temperature of the content of the flask is then maintained at 150 to 230° C. for 12 hours for performing polycondensation reaction, and then the pressure is gradually decreased at 210 to 250° C., thereby synthesizing an amorphous polyester resin (1).

The amorphous polyester resin (1) has a weight average molecular weight (Mw) of 23,200. The amorphous polyester resin (1) has an acid value of 14.2 KOHmg/g. The amorphous polyester resin (1) has a glass transition temperature (Tg) of 62° C. and a specific gravity of 1.2.

2. Production of Amorphous Binder Resin Dispersion Liquid  
20 Production of Amorphous Polyester Resin Dispersion Liquid (1)

|                                                                                                          |           |
|----------------------------------------------------------------------------------------------------------|-----------|
| Amorphous polyester resin (1)                                                                            | 100 parts |
| Solvent (1) (methyl ethyl ketone)                                                                        | 40 parts  |
| Solvent (2) (2-propanol)                                                                                 | 25 parts  |
| Basic compound (10% by weight aqueous ammonia)                                                           | 3.5 parts |
| Distilled water                                                                                          | 400 parts |
| (subjected to deoxidation by bubbling with dry nitrogen under reduced pressure before dropwise addition) |           |

The resin (1), the solvent (1) and the solvent (2) are put into a vessel, in which temperature control and nitrogen substitution may be performed, for dissolving the resin in the solvents. The basic compound is then added thereto, and the mixture is stirred with anchor blades driven by Three-One Motor (available from Shinto Scientific Co., Ltd.) at 150 rpm and 41° C. for 10 minutes, thereby providing a resin-containing liquid.

The vessel is then subjected to dry nitrogen substitution, the temperature is set at 41° C., and distilled water is added dropwise at a rate of 1 part per minute to the resin-containing liquid under stirring at 180 rpm, thereby performing phase inversion emulsification.

After completing the dropwise addition, bubbling with dry nitrogen is performed at 25° C. for 24 hours under stirring at 70 rpm, thereby removing the solvent (1) and the solvent (2), and thus the resin particle dispersion liquid (1) is obtained. The resin particles (1) in the resin particle dispersion liquid (1) have a volume average particle diameter of 210 nm. The resin particle dispersion liquid (1) has a solid concentration of 32%.

3. Production of Release Agent Dispersion Liquid

| Release Agent Dispersion Liquid                                                    |           |
|------------------------------------------------------------------------------------|-----------|
| Paraffin wax (HNP-9, available from Nippon Seiro Co., Ltd., melting point: 75° C.) | 50 parts  |
| Anionic surfactant (Neogen RK, available from Daiichi Kogyo Seiyaku Co., Ltd.)     | 0.5 part  |
| Ion exchanged water                                                                | 200 parts |

The aforementioned components are mixed and heated to 95° C., and then dispersed with a homogenizer (Ultra-Turrax T50, available from IKA Works, Inc.). Thereafter, the mixture

## 19

is dispersed with Manton Gaulin High-pressure Homogenizer (Gaulin, Inc.), thereby preparing a release agent dispersion liquid having the release agent dispersed therein (solid concentration: 20%). The release agent has a volume average particle diameter of 0.23  $\mu\text{m}$ .

## 4. Production of Colorant Dispersion Liquid

| Colorant Dispersion Liquid                                                                                                       |             |
|----------------------------------------------------------------------------------------------------------------------------------|-------------|
| Cyan pigment<br>(C.I. Pigment Blue 15:3 (copper phthalocyanine), available from Dainichiseika Colour & Chemicals Mfg. Co., Ltd.) | 1,000 parts |
| Anionic surfactant<br>(Neogen R, available from Daiichi Kogyo Seiyaku Co., Ltd.)                                                 | 15 parts    |
| Ion exchanged water                                                                                                              | 9,000 parts |

The aforementioned components are mixed and dissolved, and then dispersed with a high-pressure impact dispersing machine, Altimizer (HJP 30006, available from Sugino Machine, Ltd.) for 1 hour, thereby preparing a colorant dispersion liquid having a colorant (cyan pigment) dispersed therein. The colorant dispersion liquid has a volume average particle diameter of the colorant (cyan pigment) of 0.16  $\mu\text{m}$  and a solid concentration of 20%.

## 5. Production of Rutile Type Titanium Oxide External Additive

10 parts of rutile type titanium oxide (MT-150A, available from Tayca Corporation) having a volume average particle diameter of 15 nm, which has been rinsed with water for decreasing the amount of water soluble contents, is added to a methanol-water (95/5) mixed solvent having 1.0 part of methyltrimethoxysilane dissolved therein, and the mixture is dispersed with ultrasonic wave. The resulting dispersion liquid is then dried by evaporating methanol and the like in the dispersion liquid with an evaporator, and then the solid content is subjected to a heat treatment with a dryer set at 120  $^{\circ}\text{C}$ ., and pulverized with a mortar, thereby providing a rutile type titanium oxide external additive having a volume average particle diameter of 20 nm and a specific gravity of 4.1 having been surface-treated with methyltrimethoxysilane.

## 6. Production of Metatitanic Acid External Additive

Ilmenite as ore is dissolved in sulfuric acid, iron powder is separated, and  $\text{TiO(OH)}_2$  is produced by a wet sedimentation method where  $\text{TiO(OH)}_2$  is formed by hydrolyzing  $\text{TiOSO}_4$ . During the production of  $\text{TiO(OH)}_2$ , hydrolysis, dispersion control for formation of nuclei, and rinsing with water are performed. 100 parts of  $\text{TiO(OH)}_2$  thus obtained is dispersed in 1,000 mL of water, to which 40 parts of isobutyltrimethoxysilane is added at 40  $^{\circ}\text{C}$ . dropwise under stirring. Thereafter, the mixture is filtered and repeatedly rinsed with water. The resulting metatitanic acid particles having been subjected to a surface hydrophobic treatment are dried at 150  $^{\circ}\text{C}$ ., thereby providing a metatitanic acid external additive having a volume average particle diameter of 30 nm and a specific gravity of 3.2.

## 7. Production of Toner

## Production of Toner (1)

|                                                 |           |
|-------------------------------------------------|-----------|
| Amorphous polyester resin dispersion liquid (1) | 272 parts |
| Colorant dispersion liquid                      | 25 parts  |
| Release agent dispersion liquid                 | 40 parts  |
| Anionic surfactant                              | 2.0 parts |
| (Tayca Power, available from Tayca Corporation) |           |
| Mixing                                          |           |

## 20

The aforementioned components are put into a cylindrical stainless steel vessel and mixed with a homogenizer (Ultra-Turrax T50, available from IKA Works, Inc.) while applying a shearing force at a rotation number of the homogenizer of 4,000 rpm for 10 minutes. Thereafter, 2.0 parts of a 10% nitric acid aqueous solution of polyaluminum chloride (PAC) as an aggregating agent (nitric acid content: 0.05 N) is gradually added dropwise thereto while mixing with a homogenizer at a rotation number of 5,000 rpm over 15 minutes, thereby providing a raw material dispersion liquid.

## Aggregation

Thereafter, the raw material dispersion liquid is placed in a polymerization vessel equipped with a stirring device and a thermometer and heated by a mantle heater, and growth of aggregated particles is accelerated at 44  $^{\circ}\text{C}$ . At this time, the pH of the raw material dispersion liquid is controlled to a range of from 3.2 to 3.8 with 0.3 N nitric acid or a 1N sodium hydrochloride aqueous solution. The raw material dispersion liquid is retained for 2 hours while maintaining the pH within the range, thereby forming aggregated particles. The aggregated particles have a volume average particle diameter of 4.6  $\mu\text{m}$ .

## Coalescence

100 parts of the amorphous polyester resin dispersion liquid (1) is further added to the raw material dispersion liquid, thereby adding the resin particles of the amorphous polyester resin (1) are added to the surface of the aggregated particles. The temperature of the raw material dispersion liquid is then increased to 44  $^{\circ}\text{C}$ ., and the aggregated particles are regulated while confirming the size and shape of the particles with an optical microscope and Multisizer II. Thereafter, for coalescing the aggregated particles, the pH of the raw material dispersion liquid is adjusted to 7.0 by adding a NaOH aqueous solution dropwise thereto, and then the temperature of the raw material dispersion liquid is increased to 92  $^{\circ}\text{C}$ . Thereafter, the aggregated particles are coalesced by retaining the raw material dispersion liquid for 3 hours, and after confirming that the aggregated particles are coalesced with an optical microscope, the resulting colored particle dispersion liquid is cooled at a temperature decreasing rate of 1.0  $^{\circ}\text{C}$ . per minute.

## Rinsing

The colored particle dispersion liquid is filtered for solid-liquid separation, and the resulting colored particles are then dispersed in ion exchanged water in an amount of 20 times the amount of the solid content of the colored particles at 30  $^{\circ}\text{C}$ ., and stirred for 20 minutes, followed by filtration. The rinsing operation is repeated 5 times, and then it is confirmed that the filtrate has an electroconductivity of 22  $\mu\text{S}$ . The colored particles (1) have a volume average particle diameter of 5.4  $\mu\text{m}$  and a degree of circularity measured with FPIA-3000 of 0.968.

## Addition of Silica-Containing Particles

The colored particles dispersion liquid having been subjected to the rinsing is filtered and controlled to have a solid concentration of 35% with ion exchanged water. Hydrophobic silica particles having a diameter of 12 nm (R8200, available from Nippon Aerosil Co., Ltd., HMDS treatment) are dispersed in a mixed liquid of methanol and water at a ratio methanol/water of 50/50, and the mixture is gradually diluted with ion exchanged water, thereby controlling to provide a silica particle dispersion liquid having a solid concentration of the silica particles of 32%. The silica particle dispersion liquid is a mixed liquid of methanol and water at a ratio of 20/80. 1.78 parts by weight based on the colored particles of the silica particle dispersion liquid (corresponding to a coverage of 120%) is gradually added dropwise to the colored particles dispersion liquid under stirring. Thereafter, the pH is

decreased to 4.0 by adding 0.3 N nitric acid dropwise thereto, and the dispersion liquid is stirred for 30 minutes and then filtered. Ion exchanged water in an amount providing a solid concentration of 10% is slowly added dropwise to the resulting solid matter, and the mixture is stirred for 30 minutes and then filtered again. The resulting solid matter is put into a vacuum freeze dryer and dried at 25° C. for 24 hours, thereby providing the colored particles having the silica particles added (1).

Observation of the colored particles having the silica particles added (1) with an SEM reveals that the silica particles are added uniformly to the surface of the colored particles.

#### Dry External Addition

100 parts of the colored particles having the silica particles added (1) and 1.38 parts of rutile type titanium oxide external additive (corresponding to a coverage of 30%) are put into a Henschel mixer with a content of 5 L and mixed at a rotation number of 2,200 for 2.5 minutes. The mixture is then sieved with a 45 µm-sieve, thereby providing a toner (1). The toner (1) has an exposure ratio of 16% measured by XPS, and a contact ratio of the rutile type titanium oxide particles to the surface of the colored particles of 6% by number measured with SEM.

#### Production of Toner (2)

Colored particles (2) are produced in the same manner as for the toner (1) except that the retention time of the aggregated particles is changed to 2.5 hours, and the coalescence time thereof is changed to 3.5 hours. The colored particles (2) have a volume average particle diameter of 6.2 µm and a degree of circularity measured with FPIA-3000 of 0.972. A toner (2) is obtained in the same manner as for the toner (1) except that the amount of the hydrophobic silica particles, R8200, is changed from 1.78 parts by weight to 1.55 parts by weight (corresponding to a coverage of 120%), and the amount of the rutile type titanium oxide external additive is changed from 1.38 parts to 1.20 parts (corresponding to a coverage of 30%). The toner (2) has an exposure ratio of 14% measured by XPS, and a contact ratio of the rutile type titanium oxide particles to the surface of the colored particles of 5% by number measured with SEM.

#### Production of Toner (3)

A toner (3) is produced in the same manner as for the toner (1) except that 1.38 parts of the rutile type titanium oxide external additive (corresponding to a coverage of 30%) is changed to 1.34 parts of a metatitanic acid external additive (corresponding to a coverage of 25%). The toner (3) has an exposure ratio of 13% measured by XPS, and a contact ratio of the rutile type titanium oxide particles to the surface of the colored particles of 4% by number measured with SEM.

#### Production of Toner (4)

A toner (4) is produced in the same manner as for the toner (1) except that 1.78 parts by weight of the hydrophobic silica particles, R8200, (corresponding to a coverage of 120%) is changed to 1.36 parts by weight of the hydrophobic silica particles, R8200, (corresponding to a coverage of 92%). The toner (4) has an exposure ratio of 22% measured by XPS, and a contact ratio of the rutile type titanium oxide particles to the surface of the colored particles of 12% by number measured with SEM.

#### Production of Toner (5)

A toner (5) is produced in the same manner as for the toner (1) except that 1.78 parts by weight of the hydrophobic silica particles, R8200, (corresponding to a coverage of 120%) is changed to 2.04 parts by weight of the hydrophobic silica particles, R8200, (corresponding to a coverage of 138%). The toner (5) has an exposure ratio of 10% measured by XPS, and a contact ratio of the rutile type titanium oxide particles to the surface of the colored particles of 4% by number measured with SEM.

#### Production of Toner (6)

A silica particle dispersion liquid is produced in the same manner as for the toner (1) except that the hydrophobic silica particles, R8200, is changed to hydrophobic silica particles, R972, having a diameter of 12 nm (available from Nippon Aerosil Co., Ltd., dimethyldichlorosilane treatment). Colored particles having the silica particles added (2) are produced in the same manner as for the colored particles having the silica particles added (1) except that 2.37 parts by weight of the silica particle dispersion liquid produced herein (corresponding to a coverage of 120%) is gradually added dropwise.

Observation of the colored particles having the silica particles added (2) with an SEM reveals that the silica particles are added uniformly to the surface of the colored particles.

A toner (6) is produced in the same manner as for the toner (1) for the later procedures. The toner (6) has an exposure ratio of 14% measured by XPS, and a contact ratio of the rutile type titanium oxide particles to the surface of the colored particles of 6% by number measured with SEM.

#### Production of Toner (7)

A toner (7) is produced in the same manner as for the toner (1) except that 1.78 parts by weight of the hydrophobic silica particles, R8200, (corresponding to a coverage of 120%) is changed to 2.39 parts by weight of the hydrophobic silica particles, R8200, (corresponding to a coverage of 162%). The toner (7) has an exposure ratio of 9% measured by XPS, and a contact ratio of the rutile type titanium oxide particles to the surface of the colored particles of 4% by number measured with SEM. Portions where the silica particles are accumulated to two or more layers are found occasionally.

#### Production of Toner (8)

A toner (8) is produced in the same manner as for the toner (1) except that 1.78 parts by weight of the hydrophobic silica particles, R8200, (corresponding to a coverage of 120%) is changed to 1.18 parts by weight of the hydrophobic silica particles, R8200, (corresponding to a coverage of 80%). The toner (8) has an exposure ratio of 27% measured by XPS, and a contact ratio of the rutile type titanium oxide particles to the surface of the colored particles of 17% by number measured with SEM.

#### Production of Toner (9)

A toner (9) is produced in the same manner as for the toner (1) except that 1.78 parts by weight of the hydrophobic silica particles, R8200, (corresponding to a coverage of 120%) is added by dry external addition to the colored particles before the addition of the silica-containing particles, and then 1.38 parts of the rutile type titanium oxide external additive (corresponding to a coverage of 30%) are further added thereto by dry external addition. The toner (9) has an exposure ratio of 34% measured by XPS, and a contact ratio of the rutile type titanium oxide particles to the surface of the colored particles of 32% by number measured with SEM.

#### Example 1

The toner (1) is retained in an environment of 45° C. and 50% RH for 24 hours. The toner (1) is then installed in a modified machine of XP-15, available from Fuji Xerox Co., Ltd., (non-contact development system), and an image having an image area ratio of 10% is printed in an environment of 32° C. and 85% RH for 5,000 sheets, which are subjected to the following evaluation. The paper used for testing is recycled copier paper, G70 (available from Fuji Xerox Co., Ltd., recycled paper pulp content: 70%, basis weight: 67 g/m<sup>2</sup>, ISO whiteness: 72%).

#### Addition to Surface of Photoconductor

After printing 5,000 sheets, the additions on the photoconductor are visually observed and evaluated according the



TABLE 1-continued

|                               |                                             | Example 1   | Example 2   | Example 3        | Example 4   | Example 5   | Example 6   | Example 7   | Comparative Example 1 | Comparative Example 2 |
|-------------------------------|---------------------------------------------|-------------|-------------|------------------|-------------|-------------|-------------|-------------|-----------------------|-----------------------|
| particles                     | Addition amount (% by weight)               | 1.78        | 1.55        | 1.78             | 1.36        | 2.04        | 2.37        | 2.39        | 1.18                  | 1.78                  |
|                               | Calculated coverage (%)                     | 120         | 120         | 120              | 92          | 138         | 120         | 162         | 80                    | 120                   |
| Titanium-containing particles | Kind                                        | rutile type | rutile type | metatitanic acid | rutile type | rutile type | rutile type | rutile type | rutile type           | rutile type           |
|                               | Addition amount (% by weight)               | 1.38        | 1.20        | 1.34             | 1.38        | 1.38        | 1.38        | 1.38        | 1.38                  | 1.38                  |
|                               | Calculated coverage (%)                     | 30          | 30          | 25               | 30          | 30          | 30          | 30          | 30                    | 30                    |
|                               | Contact ratio to colored particles (%)      | 6           | 5           | 4                | 12          | 4           | 6           | 4           | 17                    | 32                    |
| Exposure ratio (%)            | Evaluation                                  | 16<br>G1    | 14<br>G1    | 13<br>G1         | 22<br>G1    | 10<br>G2    | 14<br>G1    | 9<br>G2     | 27<br>G1              | 34<br>G3              |
|                               | Addition to surface of photoconductor       |             |             |                  |             |             |             |             |                       |                       |
|                               | Image density stability                     | G1          | G1          | G1               | G2          | G1          | G1          | G1          | G3                    | G4                    |
|                               | Fogging                                     | G1          | G1          | G1               | G2          | G1          | G1          | G1          | G3                    | G4                    |
|                               | Change of minimum fixing temperature (° C.) | 3           | 3           | 3                | 5           | 4           | 3           | 5           | 7                     | 10                    |

The foregoing description of the exemplary embodiments of the present invention has been provided for the purposes of illustration and description. It is not intended to be exhaustive or to limit the invention to the precise forms disclosed. Obviously, many modifications and variations will be apparent to practitioners skilled in the art. The embodiments were chosen and described in order to best explain the principles of the invention and its practical applications, thereby enabling others skilled in the art to understand the invention for various embodiments and with the various modifications as are suited to the particular use contemplated. It is intended that the scope of the invention be defined by the following claims and their equivalents.

What is claimed is:

1. A toner for developing an electrostatic image, comprising:  
colored particles containing a colorant and a binder resin, and  
two or more kinds of inorganic particles that are externally added to the colored particles, wherein  
the two or more kinds of inorganic particles contain titanium-containing particles and silica-containing particles,  
an exposure ratio of a surface of the colored particles is about 25% or less, and  
about 15% by number or less of the titanium-containing particles are in direct contact with the colored particles.
2. The toner for developing an electrostatic image according to claim 1, wherein the exposure ratio of the surface of the colored particles is about 16% or less.
3. The toner for developing an electrostatic image according to claim 1, wherein a total of a coverage of the titanium-containing particles and a coverage of the silica-containing particles on the colored particles is about 150% or less.
4. The toner for developing an electrostatic image according to claim 1, wherein the exposure ratio of the surface of the colored particles is 2% or more.

5. The toner for developing an electrostatic image according to claim 1, wherein the silica-containing particles have a volume average particle diameter of from about 5 nm to about 40 nm.

6. The toner for developing an electrostatic image according to claim 1, wherein the titanium-containing particles have a volume average particle diameter of from about 8 nm to about 50 nm.

7. The toner for developing an electrostatic image according to claim 1, wherein a ratio of coverage of the titanium-containing particles to the silica-containing particles is from about 1/2 to about 1/10 based on the addition amounts.

8. A method of producing the toner for developing an electrostatic image according to claim 1, comprising:

preparing colored particles containing a colorant and a binder resin;  
adding silica-containing particles to the colored particles in an aqueous medium, through wet external addition to provide colored particles having the silica-containing particles added; and  
adding titanium-containing particles to the colored particles having the silica-containing particles added, through dry external addition.

9. The method of producing the toner for developing an electrostatic image according to claim 8, wherein in the addition of the silica-containing particles, an amount of the silica-containing particles in the aqueous medium is such an amount that provides a coverage on the colored particles of about 90% to about 150%.

10. The method of producing the toner for developing an electrostatic image according to claim 8, wherein a total of a coverage of the titanium-containing particles and a coverage of the silica-containing particles on the colored particles is about 150% or less.

11. The method of producing the toner for developing an electrostatic image according to claim 8, wherein an exposure ratio of a surface of the colored particles is about 2% or more.

12. An image forming method comprising:  
forming an electrostatic latent image on a surface of an image holding member;  
developing the electrostatic latent image formed on the surface of the image holding member, with a toner, to form a toner image;

**27**

transferring the toner image to a surface of a transfer medium; and  
fixing the toner image transferred to the surface of the transfer medium,  
wherein the toner is the toner for developing an electro- 5  
static image according to claim 1.

**13.** The image forming method according to claim 12,  
wherein a total of a coverage of the titanium-containing particles and a coverage of the silica-containing particles on the colored particles is about 150% or less. 10

**14.** The image forming method according to claim 12,  
wherein the exposure ratio of the surface of the colored particles is about 2% or more.

**15.** The toner for developing an electrostatic image according to claim 1, wherein the silica-containing particles have a 15  
volume average particle diameter of from 7 nm to 30 nm.

**28**

\* \* \* \* \*